

# United States Patent

Plapper et al.

[15] 3,661,631

[45] May 9, 1972

[54] **METHOD FOR IMPARTING WATER- AND OIL-REPELLENT PROPERTIES TO LEATHER AND LEATHER SO TREATED**

[72] Inventors: **Jurgen Plapper**, Dusseldorf-Holthausen; **Friedrich Pieper**, Langenfeld-Richrath, both of Germany

[73] Assignee: **Henkel & Cie GmbH**, Dusseldorf Holthausen, Germany

[22] Filed: **June 18, 1970**

[21] Appl. No.: **47,593**

[30] **Foreign Application Priority Data**

June 27, 1969 Germany .....P 19 32 630.8

[52] U.S. Cl. .... **117/142, 252/8.57**

[51] Int. Cl. .... **B44d 1/32, C14c 7/00**

[58] Field of Search ..... **252/8.57; 117/142**

[56] **References Cited**

UNITED STATES PATENTS

|           |         |                |                |
|-----------|---------|----------------|----------------|
| 3,106,478 | 10/1963 | Heyden et al.  | .....117/142 X |
| 3,019,133 | 1/1962  | Heyden et al.  | .....117/142   |
| 3,524,760 | 8/1970  | Pinkerton      | .....117/142 X |
| 3,527,742 | 9/1970  | Pittman et al. | .....117/142 X |
| 2,953,479 | 9/1960  | Heyden et al.  | .....117/135.5 |

|           |         |                |                 |
|-----------|---------|----------------|-----------------|
| 2,977,249 | 3/1961  | Heyden et al.  | .....117/135.5  |
| 3,471,518 | 10/1969 | Hager          | .....252/8.57 X |
| 3,409,647 | 11/1968 | Pittman et al. | .....252/8.57 X |
| 3,501,448 | 3/1970  | Pittman et al. | .....117/142 X  |

FOREIGN PATENTS OR APPLICATIONS

824,436 12/1959 Great Britain .....252/8.57

Primary Examiner—William D. Martin  
Assistant Examiner—Harry J. Ginnell  
Attorney—Hammond & Littell

[57] **ABSTRACT**

A method for imparting water- and oil-repellent properties to leather is disclosed which uses as the treating composition a solution of

a. a condensation product formed by (1) an aluminum alcoholate of a lower monohydroxy alcohol having a carbon chain length of one to four carbon atoms with (2) a phosphoric acid monoester of a higher fatty alcohol having a carbon chain length of 12 to 20 carbon atoms, and

b. a fluorinated compound comprising lipophilic radicals having a carbon chain length of eight to 20 carbon atoms, selected from the group consisting of fluorocarboxylic acids and esters thereof, and fluoroalcohols and esters, ethers and acetals thereof in an inert organic solvent; the solution is applied to dry leather by immersion or spraying, as well as the water- and oil-repellent leather so produced.

16 Claims, No Drawings

**METHOD FOR IMPARTING WATER- AND OIL-REPELLENT PROPERTIES TO LEATHER AND LEATHER SO TREATED**

**THE PRIOR ART**

From German Pat. No. 1,061,478 the use of condensation products of alcoholates of multivalent metals and acid higher-molecular organic derivatives of the phosphoric acids in organic solvents for the impregnation of leather is known. The impregnation imparts water-repellent characteristics to the leather, especially good water-repellent effects being achieved and the absorption of water of the impregnated leathers is also reduced to a greater or less extent. At greater concentrations, however, the leathers become increasingly hardened and of a darker coloration, while the water absorption and the dynamic water resistance are increased only slightly.

The use of so-called fluoro-chemicals for the leather impregnation is also known. Such fluoro-chemicals include saturated or unsaturated fluorocarboxylic acids and fluorocarcohols of chain lengths  $C_8$  to  $C_{18}$  and their esters and derivatives, as well as polymerizable fluorine-containing compounds such as for instance acrylic or methacrylic esters of fluorinated higher alcohols or esters and ethers of allyl alcohol with fluorinated higher carboxylic acids or alcohols or acetals of unsaturated aldehydes with fluorinated alcohols, etc.

In the impregnation with the fluoro-chemicals in organic solution, water and oil repellent leathers are obtained which show good water-repellent and oil-repellent effects. The dynamic water resistance is no better, however, than in the leathers impregnated with phosphoric acid ester condensation products. It is true that increasing the concentration of the fluoro-chemicals applied reduces the water absorption but the characteristics of the leather deteriorate increasingly at the same time. The leathers become harder and more speckled. Furthermore, at increasing concentrations the oil-repellent effect is increasingly reduced.

**OBJECTS OF THE INVENTION**

It is the object of the invention to achieve a better full impregnation and better water characteristic, especially a better dynamic water resistance of the impregnated leather, without any deterioration in the general character of the leather through hardening, spotting or discoloration.

Another object of the present invention is the development of a process for imparting water- and oil-repellent properties to leather which comprises impregnating a dry leather with an inert organic solvent solution containing from 0.5 percent to 6 percent by weight of a mixture of (A) from about 10 percent to 95 percent by weight of the condensation product of an aluminum alcoholate of an alkanol having from one to four carbon atoms with a phosphoric acid monoester of an alkanol having from 12 to 20 carbon atoms in a molar ratio of from 1:0.5 to 1:1.5 and (B) from about 5 percent to 90 percent by weight of a fluorinated lipophilic compound having from eight to 20 carbon atoms selected from the group consisting of higher saturated and unsaturated fluorocarboxylic acids and their esters with lower alkanols and lower alkenols, higher saturated and unsaturated fluorocarcohols, their esters with lower alkanols and lower alkenols and their acetals with lower alkanals and lower alkenals, higher saturated and unsaturated fluorocaralcohols, their esters with lower alkanols and lower alkenols and their acetals with lower alkanals and lower alkenals, drying said impregnated leather at temperatures from room temperature to about 70°C and recovering a leather having water- and oil-repellent properties.

A further object of the invention is the obtaining of an inert organic solvent solution for impregnating leather to impart water- and oil-repellent properties thereto which contains from 0.5 percent to about 50 percent by weight of a mixture of (A) from about 10 percent to 95 percent by weight of the condensation products of an aluminum alcoholate of an alkanol having from one to four carbon atoms with a phosphoric acid monoester of an alkanol having from 12 to 20 carbon atoms in a molar ratio of from 1:0.5 to 1:1.5 and (B) from about 5 per-

cent to 90 percent by weight of a fluorinated lipophilic compound having from eight to 20 carbon atoms selected from the group consisting of higher saturated and unsaturated fluorocarboxylic acids and their esters with lower alkanols and lower alkenols, higher saturated and unsaturated fluorocarcohols, their esters with lower alkanols and lower alkenols and their acetals with lower alkanals and lower alkenals.

- 10 A yet further object of the invention is the production of a leather having water- and oil-repellent properties having a surface impregnation of from about 1 gm/m<sup>2</sup> to about 14 gm/m<sup>2</sup> of leather surface of a mixture of (A) from about 10 percent to 95 percent by weight of the condensation product of an aluminum alcoholate of an alkanol having from one to four carbon atoms with a phosphoric acid monoester of an alkanol having from 12 to 20 carbon atoms in a molar ratio of from 1:0.5 to 1:1.5 and (B) from about 5 percent to 90 percent by weight of a fluorinated lipophilic compound having from eight to 20 carbon atoms selected from the group consisting of higher saturated and unsaturated fluorocarboxylic acids and their esters with lower alkanols and lower alkenols, higher saturated and unsaturated fluorocarcohols, their esters with lower alkanols and lower alkenols and their acetals with lower alkanals and lower alkenals.
- 15 20 25

These and other objects of the invention will become more apparent as the description thereof proceeds.

**DESCRIPTION OF THE INVENTION**

The present invention, therefore, provides a process for the impregnation of leather, comprising contacting the leather with an inert organic solvent solution having a content of:

- 30 35 A condensation product of an aluminum alcoholate of a lower mono-alcohol of chain length  $C_1$  to  $C_4$  with a phosphoric acid monoester of a higher fatty alcohol of chain length  $C_{12}$  to  $C_{20}$ , and
- 40 B. A fluoro-carboxylic acid or an ester thereof, or a fluoro-alcohol or an ester, ether or acetal thereof, which has a fluorinated lipophile residue having a chain length of  $C_8$  to  $C_{20}$ .
- 45 In a further aspect, the present invention provides a composition which comprises an inert organic solvent solution of:
- 45 50 A. A condensation product of an aluminum alcoholate of a lower mono-alcohol of chain lengths  $C_1$  to  $C_4$  with a phosphoric acid monoester of a higher fatty alcohol of chain lengths  $C_{12}$  to  $C_{20}$ , and
- 50 B. A fluoro-carboxylic acid or an ester thereof, or a fluoro-alcohol or an ester, ether or acetal thereof, which has a fluorinated lipophile residue having a chain length of  $C_8$  to  $C_{20}$  in an organic solvent.

55 It has now been found surprisingly that the combination of the components A and B which are known per se, prevents the disadvantages which are present when the two impregnating components are used separately. A better penetrating impregnation and a substantially better water resistant character of the impregnated leather is achieved, without any deterioration of the general character of the leather through hardening, spotting, discoloration etc. A further advantage is that the concentration of the active solutions applied can be substantially increased which allows further improvements, in respect of water and oil-repellent effects and of the water resistance of the impregnated leather to be achieved without substantial alteration of the character of the leather.

- 60 65 70 75 More particularly, and as a further aspect of the present invention, the invention comprises a leather having water- and oil-repellent properties having a surface impregnation of from about 1 gm/m<sup>2</sup> to about 14 gm/m<sup>2</sup> of leather surface of a mixture of (A) from about 10 percent to 95 percent by weight of the condensation product of an aluminum alcoholate of an alkanol having from one to four carbon atoms with a phosphoric acid monoester of an alkanol having from 12 to 20 carbon atoms in a molar ratio of from 1:0.5 to 1:1.5 and (B) from

about 5 percent to 90 percent by weight of a fluorinated lipophilic compound having from eight to 20 carbon atoms selected from the group consisting of higher saturated and unsaturated fluoro-carboxylic acids and their esters with lower alkanols and lower alkenols, higher saturated and unsaturated fluoro-alcohols, their esters with lower alkanols and lower alkenols, their ethers with lower alkanols and lower alkenols and their acetals with lower alkanols and lower alkenols.

The condensation products of component A are obtained according to German Pat. No. 1,061,478 by the reaction of aluminum alcoholates, such as aluminum isopropylate or butylate with phosphoric acid monoesters of higher fatty alcohols with 12 to 20 carbon atoms. The reaction is effected by bringing together the starting components in solution in an organic solvent such as isopropanol, trichloroethylene or toluene and heating, if necessary, to temperatures of from about 30° to 50° C. The molar ratio of alcoholate to phosphoric acid ester should be approximately 1:0.5 to 1.5. Up to 30 mol percent of phosphoric acid monoester may be replaced by the corresponding phosphoric acid diester of higher fatty alcohols. Suitable products of component A are the reaction product of 1 mol of aluminum isopropylate with 0.7 mols of a monoalkyl phosphoric acid ester with an alkyl having 12 to 18 carbon atoms, the reaction product of 1 mol of aluminum propylate with 0.9 mols of monotetradecyl phosphoric acid ester, the reaction product of 1 mol of aluminum butylate with 0.6 mols of a monoalkylphosphate acid ester with an alkyl having 16 to 18 carbon atoms. For stabilization before use against the effects of moisture, compounds containing enol groups, such as acetyl acetone and ethyl acetoacetate, may be added to the solutions of these products.

The compounds of component B contain as a common characteristic a lipophile fluorinated hydrocarbon residue of chain lengths  $C_8$  to  $C_{20}$ . The compounds concerned are known compounds from the group of the higher saturated or unsaturated fluoro-carboxylic acids or their esters with lower saturated or unsaturated alcohols, preferably allyl alcohol, as well as from the group of the higher saturated or unsaturated or branch-chained fluoro-alcohols and their esters, ethers or acetals with lower, preferably unsaturated carboxylic acids, alcohols or aldehydes. The following are examples of compounds of component B; perfluorodecane carboxylic acid, a mixture of perfluorinated carboxylic acids of chain lengths  $C_{12}$  to  $C_{18}$ , perfluorooctane carboxylic acid allyl ester, perfluorododecyl alcohol, perfluorododecyl alcohol acrylic acid ester, a mixture of the methacrylic acid esters of perfluorinated fatty alcohols of chain lengths  $C_{12}$  to  $C_{18}$ , perfluorododecanol formaldehyde acetal. In as far as the aforementioned compounds are esters of acrylic or methacrylic acid, or esters or ethers of allyl alcohol, the compounds are able to polymerize and may also be used in the form of their soluble polymers or copolymers.

The proportion of fluorinated compounds in the mixture of active components may be from 5 percent to 90 percent, preferably 10 percent to 50 percent by weight. Favorable effects can be achieved already with relatively small proportions of fluoro-compounds, so that the claimed process is particularly advantageous also from an economic point of view.

The products are applied in accordance with the present invention, in organic solution in concentrations of approximately 0.5 to 6 percent by weight, preferably 1 percent to 4 percent

by weight, related to the sum of components A and B. After impregnating, the leather contains from about 1 gm/m<sup>2</sup> to 14 gm/m<sup>2</sup> of leather surface of the mixture of components A and B. Possible inert organic solvents and diluents are chiefly gasolines of boiling ranges between 60° and 200° C, ethyl acetate, butyl acetate, chlorohydrocarbons such as methylene chloride, methyl chloroform, trichloroethylene, perchloroethylene, toluene, etc. and preferably mixture of gasolines of a boiling range of 60° to 95° C and ethyl acetate.

10 The treatment of the leather may be effected by immersion, but mainly however by spraying onto the surface of the leather. The leathers are treated appropriately in a dry condition. After impregnation, an after-drying at 50° to 70° C, possibly in the presence of atmospheric moisture takes place, whereupon optimum water resistance is achieved immediately. Favorable effects can also be achieved by after-drying at room temperature, but this method requires a storing period of a few days.

15 20 Specially suitable for the impregnation in accordance with the invention are types of suede leather such as shoe and clothing suedes, but also non-finished or slightly finished types of leather, such as the so-called aniline leathers.

25 The combinations of active components may contain furthermore the usual additives such as waxes, resins or dyes, so as to obtain a favorable effect on the leather character in accordance with the different types of leather. For a further increase of the water resistance commercial silicone oils on the basis of dimethyl polysiloxanes or methyl hydrogen polysiloxanes may be added to the impregnating solvent mixture in amounts of from about 0.03 to 0.4 percent by weight.

30 35 40 45 50 55 60 The following examples are illustrative of the practice of the invention without being deemed limitative in any respect.

## EXAMPLES

Stock solutions are prepared of an aluminum alcoholate phosphoric acid ester condensation product ("solution A") and a mixture of fluorinated compounds ("solution B"), from which by mixing and further dilution the impregnating solutions of the following examples are obtained.

### Solution A

216 parts by weight of aluminum isopropylate are dissolved in 240 parts by weight of perchloroethylene at elevated temperature and combined gradually with heating to 65° to 70° C and stirring with a solution of 200 parts by weight of a monoalkyl phosphoric acid ester mixture of chain lengths  $C_{12}$  to  $C_{18}$  in 200 parts by weight of perchloroethylene. To the clear solution of the reaction mixture are added 144 parts by weight of ethyl acetate with stirring and the mixture is stirred for a further 2 hours at approximately 70° C. The solution contains approximately 40 parts by weight of the aluminum alcoholate-phosphoric acid ester condensation product.

### Solution B

4.5 parts by weight of a mixture of approximately 1 part by weight of perfluorooctane carboxylic acid and approximately 2 parts by weight of the methacrylic acid ester of a fluorinated unsaturated fatty alcohol mixture of average chain length  $C_8$  are dissolved in methyl chloroform.

## EXAMPLE 1

To 32 parts by weight of solution A are added 40 parts by weight of solution B. The yellow, clear impregnating agent sol-

| Concentration applied, related to active substance, percent | Drip test |                 | Penetrometer Test: Water penetration. Average from 3 tests | Percent water absorption according to Kubelka after— |        |         | Characterization of the leather                                   |
|-------------------------------------------------------------|-----------|-----------------|------------------------------------------------------------|------------------------------------------------------|--------|---------|-------------------------------------------------------------------|
|                                                             | Water     | Machine oil     |                                                            | 30 min.                                              | 2 hrs. | 24 hrs. |                                                                   |
| Example 1.....                                              | 1         | 40 minutes...   | 40 minutes...                                              | 12 minutes...                                        | 46.1   | 59.8    | 80.3 Good handle.                                                 |
|                                                             | 4         | >1 hour.....    | >24 hours...                                               | 25 minutes.....                                      | 42.8   | 54.7    | 70.1 Slightly more greasy than with 1% active substance.          |
| Solution B.....                                             | 1         | >1 hour.....    | >24 hours...                                               | 6 minutes.....                                       | 58.1   | 70.9    | 87.1 Leather somewhat harder.                                     |
|                                                             | 4         | 30 minutes..... | No effect at high concentr.                                | 12 minutes.....                                      | 46.9   | 60.1    | 82.3 Leather hard and unattractive, spotted.                      |
| Dimethylsil-oxane.....                                      | 4         | >1 hour.....    | do.....                                                    | 7 minutes.....                                       | 60.2   | 72.3    | 93.1 No change against untreated.                                 |
| Solution A.....                                             | 4         | do.....         | do.....                                                    | 12 minutes.....                                      | 56.0   | 64.1    | 81.7 After bulling, tendency to greasiness.                       |
| Untreated leather.....                                      | 4         | minutes.....    | 2 minutes.....                                             | 115.4                                                | 119.0  | 131.0   | Leather becomes coarser and harder. Character of aniline leather. |

vent mixture is diluted with further 21 parts by weight of a gasoline of boiling range 110° to 140° C and 7 parts by weight of butyl acetate. The approximately 15 percent solution of active substance produced is further diluted before the application to the leather with a gasoline of boiling range 60° to 95° C or ethyl acetate to give a content of active substances of 1 percent and 4 percent by weight respectively.

A commercial, lightly retanned and dubbed chrome neat's upper leather of the so-called aniline leather type is sprayed with 1 percent and 4 percent respectively active substance solution of the above-mentioned impregnating agent, so that in the first case approximately 2.5 gm/m<sup>2</sup> of leather surface, and in the second case approximately 9 gm/m<sup>2</sup> of leather surface are applied. After drying and maturing of the leather, the impregnating data given in the following table were obtained. The table also contains data which was obtained with solution A and with solution B respectively after appropriate dilution and with a dimethylpolysiloxane solution of appropriate concentration and with untreated leather.

The result clearly indicates that with the impregnating agents in accordance with the invention, without detrimental changes in the character of the leather, substantially better impregnating effects were obtained than with the individual components or with commercial dimethyl-polysiloxane.

#### EXAMPLE 2

To 28 parts by weight of solution A are added 36 parts by weight of solution B and 4 parts by weight of a commercial

5 A commercial, lightly retanned and dubbed chrome neat's upper leather of the aniline leather type, is treated as described in Example 1, with the above-mentioned impregnating agent and finished. The impregnating data are to be found in the following table. In spite of the relatively small quantity of fluoro-compounds in the impregnating agent mixture a total effect much superior to that of the individual components is achieved.

10

#### EXAMPLE 3

15 To 30 parts by weight of solution A are added 60 parts by weight of solution B and the mixture is diluted with 10 parts by weight of butyl acetate. The yellow clear impregnating solution contains a proportion of active substance of approximately 15 percent by weight.

20 As described in Example 1, a commercial clothing suede of split cowhide is sprayed in dry condition with a 1 percent and 4 percent solution of active substance obtained by dilution of the above-mentioned solution with a gasoline fraction having the boiling range 60° to 95° or ethylacetate. After drying and maturing of the leather, a superior impregnating effect of the 25 mixture in accordance with the invention was discovered as compared with the individual components, as shown by the following table. No deterioration of the character of the leather was established.

| Concentration applied, related to active substance, percent | Drip test    |                                 | Penetrometer Test: Water penetration. Average from 3 tests | Percent water absorption according to Kubelka after— |        |         | Characterization of the leather         |
|-------------------------------------------------------------|--------------|---------------------------------|------------------------------------------------------------|------------------------------------------------------|--------|---------|-----------------------------------------|
|                                                             | Water        | Machine oil                     |                                                            | 30 min.                                              | 2 hrs. | 24 hrs. |                                         |
| Example 3                                                   | 1 >1 hour    | 10 minutes                      | 5 minutes                                                  | 90.3                                                 | 96.4   | 103.1   | No change against untreated.            |
|                                                             | 4 do         | >24 hours                       | 54 minutes                                                 | 57.4                                                 | 71.4   | 87.1    | No change.                              |
| Solution B                                                  | 1 >1 hour    | >24 hours                       | 6 minutes                                                  | 107.8                                                | 122.8  | 132.0   | Leather somewhat harder.                |
|                                                             | 4 30 minutes | No effect at too high concentr. | 12 minutes                                                 | 65.2                                                 | 80.0   | 100.5   | Leather hard and unattractive, spotted. |
| Dimethylsiloxane Solution A                                 | 4 >1 hour    |                                 | 7 minutes                                                  | 126.8                                                | 140.3  | 148.1   | No change against untreated.            |
|                                                             | 4 do         |                                 | 12 minutes                                                 | 91.7                                                 | 122.9  | 131.0   | After buffing, tendency to greasiness.  |
| Untreated leather                                           | 4 minutes    |                                 | 2 minutes                                                  | 137.5                                                | 142.1  | 148.4   | Leather rougher and harder.             |
|                                                             |              |                                 |                                                            |                                                      |        |         | Leather velvety dry.                    |

dimethylpolysiloxane with slight heating. The mixture is diluted with 28 parts by weight of butyl acetate and 4 parts by weight of perchloroethylene. An impregnating solution is obtained which contains approximately 17 percent by weight of active substances and which is diluted further for the application with a gasoline of boiling range 60° to 95° C or ethylacetate to give a solution having a content of active sub-

45 To 28 parts by weight of solution A are added 36 parts by weight of solution B and 4 parts by weight of dimethylpolysiloxane, 28 parts by weight of butylacetate and 4 parts by weight of perchloroethylene while heating slightly. A yellow clear impregnating solution with a content of active substance of approximately 17 percent by weight is obtained.

| Concentration applied, related to active substance, percent | Drip test    |                                 | Penetrometer Test: Water penetration. Average from 3 tests | Percent water absorption according to Kubelka after— |        |         | Characterization of the leather         |
|-------------------------------------------------------------|--------------|---------------------------------|------------------------------------------------------------|------------------------------------------------------|--------|---------|-----------------------------------------|
|                                                             | Water        | Machine oil                     |                                                            | 30 min.                                              | 2 hrs. | 24 hrs. |                                         |
| Example 4                                                   | 1 >1 hour    | 5 minutes                       | 3 minutes                                                  | 101.5                                                | 107.8  | 116.0   | No change to untreated.                 |
|                                                             | 4 do         | >24 hours                       | 75 minutes                                                 | 32.9                                                 | 56.1   | 85.0    | Do.                                     |
| Solution B                                                  | 1 >1 hour    | >24 hours                       | 6 minutes                                                  | 107.8                                                | 122.8  | 132.0   | Leather somewhat harder.                |
|                                                             | 4 30 minutes | No effect at too high concentr. | 12 minutes                                                 | 65.2                                                 | 80.0   | 100.5   | Leather hard and unattractive, spotted. |
| Dimethylsiloxane Solution A                                 | 4 >1 hour    |                                 | 7 minutes                                                  | 126.8                                                | 140.3  | 148.1   | No change to untreated.                 |
|                                                             | 4 do         |                                 | 12 minutes                                                 | 91.7                                                 | 122.9  | 134.0   | After buffing, tendency to greasiness.  |
| Untreated leather                                           | 4 minutes    |                                 | 2 minutes                                                  | 137.5                                                | 142.1  | 148.4   | Leather coarser and harder.             |
|                                                             |              |                                 |                                                            |                                                      |        |         | Leather velvety like, dry.              |

stance of approximately 1 percent and 4 percent by weight respectively.

A commercial clothing suede is sprayed as in Example 1 with an active substance solution of the above-mentioned im-

| Concentration applied, related to active substance, percent | Drip test    |                                 | Penetrometer Test: Water penetration. Average from 3 tests | Percent water absorption according to Kubelka after— |        |         | Characterization of the leather                     |
|-------------------------------------------------------------|--------------|---------------------------------|------------------------------------------------------------|------------------------------------------------------|--------|---------|-----------------------------------------------------|
|                                                             | Water        | Machine oil                     |                                                            | 30 min.                                              | 2 hrs. | 24 hrs. |                                                     |
| Example 2                                                   | 1 >1 hour    | 25 minutes                      | 5 minutes                                                  | 55.5                                                 | 68.5   | 88.1    | Good handle.                                        |
|                                                             | 4 do         | >24 hours                       | 15 minutes                                                 | 53.4                                                 | 64.0   | 81.9    | Slightly more greasy than with 1% active substance. |
| Solution B                                                  | 1 >1 hour    | >24 hours                       | 6 minutes                                                  | 58.1                                                 | 70.9   | 87.1    | Leather somewhat harder.                            |
|                                                             | 4 30 minutes | No effect at too high concentr. | 12 minutes                                                 | 46.9                                                 | 60.1   | 82.3    | Leather hard and unattractive, spotted.             |
| Dimethyl siloxane Solution A                                | 4 >1 hour    |                                 | 7 minutes                                                  | 60.2                                                 | 72.3   | 93.1    | No change against untreated.                        |
|                                                             | 4 do         |                                 | 12 minutes                                                 | 56.0                                                 | 64.1   | 81.7    | After buffing tendency to greasiness.               |
| Untreated leather                                           | 4 minutes    |                                 | 2 minutes                                                  | 115.4                                                | 119.0  | 131.0   | Leather becomes rougher and harder.                 |
|                                                             |              |                                 |                                                            |                                                      |        |         | Character of aniline leather.                       |

pregnating agent adjusted to 1 to 4 percent by weight.

After drying and maturing of the leather, an impregnating effect was obtained which was superior compared with that of the individual components, without any deterioration of the character of the leather.

The preceding specific embodiments are illustrative of the practice of the invention. It is to be understood, however, that the same is not limitative and that other expedients known to those skilled in the art may be practiced without departing from the spirit of the invention or the scope of the appended claims.

We claim:

1. A process for imparting water- and oil-repellent properties to leather which comprises impregnating a dry leather with an inert organic solvent solution containing from 0.5 percent to 6 percent by weight of a mixture of (A) from about 10 percent to 95 percent by weight of the condensation product of an aluminum alcoholate of an alkanol having from one to four carbon atoms with a phosphoric acid monoester of an alkanol having from 12 to 20 carbon atoms in a molar ratio of from 1:0.5 to 1:1.5 and (B) from about 5 percent to 90 percent by weight of a fluorinated lipophilic compound having from eight to 20 carbon atoms selected from the group consisting of higher saturated and unsaturated fluoro-carboxylic acids and their esters with lower alkanols and lower alkenols, higher saturated and unsaturated fluoro-alcohols, their esters with lower alkanoic and lower alkenoic acids, their ethers with lower alkanols and lower alkenols and their acetals with lower alkanals and lower alkenals, drying said impregnated leather at temperatures from room temperature to about 70° C and recovering a leather having water- and oil-repellent properties.

2. The process of claim 1 wherein said component A is a condensation product of aluminum isopropylate with from 0.7 to 1.5 mols of a monoalkyl phosphoric acid ester having from 12 to 18 carbon atoms in the alkyl.

3. The process of claim 1 wherein said component B is a mixture of perfluorooctane carboxylic acid and a methacrylic acid ester of a fluorinated unsaturated fatty alcohol having an average of 8 carbon atoms.

4. The process of claim 1 wherein said component A is present in an amount of from 50 to 90 percent by weight and said component B is present in an amount of from 10 to 50 percent by weight in said mixture.

5. The process of claim 1 wherein said inert organic solvent is selected from the group consisting of gasoline fractions having boiling ranges between 60° C and 200° C, ethyl acetate, butyl acetate, trichloroethylene and toluene.

6. The process of claim 1 wherein the concentration of said mixture in said solution is from 1 to 4 percent by weight.

7. The process of claim 1 wherein said organic solvent solution contains from 0.03 to 0.4 percent by weight of a polysiloxane selected from the group consisting of dimethylpolysiloxanes and methyl hydrogen polysiloxanes.

8. The process of claim 1 wherein said organic solvent solution contains a content of an enolic compound as a stabilizer against moisture.

9. The process of claim 8 wherein said enolic compound is

present in an amount of 1 mol per mol of component A and is selected from the group consisting of acetyl acetone and ethyl acetoacetate.

10. An inert organic solvent solution for impregnating leather to impart water- and oil-repellent properties thereto which contains from 0.5 to about 50 percent by weight of a mixture of (A) from about 10 to 95 percent by weight of the condensation product of an aluminum alcoholate of an alkanol having from one to four carbon atoms with a phosphoric acid monoester of an alkanol having from 12 to 20 carbon atoms in a molar ratio of from 1:0.5 to 1:1.5 and (B) from about 5 to 90 percent by weight of a fluorinated lipophilic compound having from eight to 20 carbon atoms selected from the group consisting of higher saturated and unsaturated fluoro-carboxylic acids and their esters with lower alkanols and lower alkenols, higher saturated and unsaturated fluoro-alcohols, their esters with lower alkanoic and lower alkenoic acids, their ethers with lower alkanols and lower alkenols and their acetals with lower alkanals and lower alkenals.
11. The inert organic solvent solution of claim 10 wherein said component A is a condensation product of aluminum isopropylate with from 0.7 to 1.5 mols of a monoalkyl phosphoric acid ester having from 12 to 18 carbon atoms in the alkyl.
12. The inert organic solvent solution of claim 10 wherein said component B is a mixture of perfluorooctane carboxylic acid and a methacrylic acid ester of a fluorinated unsaturated fatty alcohol having an average of eight carbon atoms.
13. The inert organic solvent solution of claim 10 wherein said component A is present in an amount of from 50 to 90 percent by weight and said component B is present in an amount of from 10 to 50 percent by weight in said mixture.
14. The inert organic solvent solution of claim 10 wherein said inert organic solvent is selected from the group consisting of gasoline fractions having boiling ranges between 60° C and 200° C, ethyl acetate, butyl acetate, trichloroethylene and toluene.
15. The inert organic solvent solution of claim 10 wherein the concentration of said mixture in said solution is from 1 to 4 percent by weight.
16. A leather having water- and oil-repellent properties having a surface impregnation of from about 1 gm/m<sup>2</sup> to about 14 gm/m<sup>2</sup> of leather surface of a mixture of (A) from about 10 to 95 percent by weight of the condensation product of an aluminum alcoholate of an alkanol having from one to four carbon atoms with a phosphoric acid monoester of an alkanol having from 12 to 20 carbon atoms in a molar ratio of from 1:0.5 to 1:1.5 and (B) from about 5 to 90 percent by weight of a fluorinated lipophilic compound having from eight to 20 carbon atoms selected from the group consisting of higher saturated and unsaturated fluoro-carboxylic acids and their esters with lower alkanols and lower alkenols, higher saturated and unsaturated fluoro-alcohols, their esters with lower alkanoic and lower alkenoic acids, their ethers with lower alkanols and lower alkenols and their acetals with lower alkanals and lower alkenals.

\* \* \* \* \*